

Dec. 8, 1942.

M. O. SCHUR

2,304,287

MANUFACTURE OF GREASE-RESISTANT PAPER

Filed March 23, 1939



Fig. 1.



Fig. 2.

Inventors  
Milton O. Schur  
Arthur W. Wishart  
By Nathaniel P. Harton  
Atty.

## UNITED STATES PATENT OFFICE

2,304,287

MANUFACTURE OF GREASE-RESISTANT  
PAPER

Milton O. Schur, Berlin, N. H., assignor, by mesne assignments, to Reconstruction Finance Corporation, Washington, D. C., a corporation of the United States of America

Application March 23, 1939, Serial No. 263,664

13 Claims. (Cl. 117—83)

This invention relates to the manufacture of grease-resistant paper and more especially of paper such as is to serve in the food-wrapping and food-packaging art for such purposes as lining bags, boxes, or other containers for greasy or oily comestibles of the nature of coffee, cocoa, peanuts, potato chips, cookies, crackers, etc. The grease-resistant or greaseproof paper product hereof may be used to advantage as a liner in an ordinary paper bag or in a box or container of the usual paperboard variety. It may also be used by itself, that is, without an external wrapping, bag, or container, as a food-wrapping or food-packaging medium.

Such grease-resistant papers as have heretofore been available for food-wrapping or food-packaging purposes are quite expensive. This is especially true of parchment paper and is also true of glassine paper, which latter paper is so brittle and deficient in flex-endurance and tear-resistance as to be apt to be fractured or torn during machine-fabrication or filling of the package or once the package in which it serves as a liner has been opened and the liner is exposed to handling.

The present invention provides at comparatively low cost a greaseproof paper product that is not only serviceable in lieu of glassine and parchment papers in the food-wrapping and food-packaging art but that is also characterized by much higher flex-endurance and tear-resistance than glassine paper. As an illustration, the greaseproof paper product hereof may be supplied to bakeries, wherein it may advantageously replace the more expensive glassine paper for lining the paperboard boxes in which shortened crackers, cookies, and other bakery products are packed and sold. As another illustration, the greaseproof paper product hereof may be sold to coffee-packing establishments, wherein it may be used instead of the more expensive greaseproof papers heretofore used in making the liner bag of a two-ply paper bag for holding and vending coffee. Indeed, if the outer coffee bag is prepared from paper according to the present invention, the inner bag may be dispensed with, thereby lending a substantial saving in the cost of the package.

In producing the greaseproof paper product hereof, an ordinary non-grease-resistant paper base, such as bleached or unbleached kraft paper, may serve as the starting material. The paper base, which may contain, if desired, a small amount of such usual sizing material as rosin, starch, or the like, is preferably primed on at

least one surface with a composition containing bentonite and preferably also a suitable binder, such as cooked starch, casein, glue, etc. After the paper surface has been primed with an aqueous priming composition containing bentonite and water-soluble binder and the primed surface has been dried, the resulting primed surface is coated with zein or equivalent grease-resistant prolamine in the form of a solution in a suitable 5 volatile organic solvent, such as ethyl alcohol, and the coated surface dried. Only an extremely thin coating of the zein on the preferably bentonite-primed paper surface is necessary for developing a finished paper product of remarkably 10 high grease-resistance.

The priming of the paper surface with bentonite composition is preferred in that it facilitates the realization of the desired grease-resistant or grease-proof paper product hereof. 15 Thus, when priming of the paper surface is effected with other filling or priming compositions, such as compositions containing ordinary clay, talc, calcium carbonate, or the like, it is much 20 more difficult to produce a paper product of uniformly satisfactory greaseproof quality unless so much zein is subsequently applied as a coating to the primed surface as to render less feasible 25 economically the manufacture of a paper product competitive with glassine paper. It is evidently the case that the colloidal clay known as bentonite is outstanding in its ability to deposit within the pores on a normal paper surface a 30 priming film of such tightness, continuity, or fine texture that it can take on a very thin zein 35 coating practically free from such gaps, disruptions, or pinholes as would detract seriously from or vitiate the greaseproof quality desired in the finished paper product. Again, the desired 40 greaseproof quality is attained in the finished paper product hereof while using only such small amount of bentonite as priming material as does not detract materially from the flex-enduring 45 and tear-resisting qualities (per unit of overall weight) characteristic of the original paper base, which is very much more like an ordinary paper base in such latter qualities than like glassine paper. Along with the bentonite as the priming substance, it is preferred to use cooked starch as the binder, for the combination of bentonite and cooked starch in the priming composition 50 has been found to give excellent results. Thus, a priming composition containing bentonite and cooked potato starch has been found to be much better for the purposes hereof than a priming

composition containing bentonite and such other binders as casein, glue, etc.

While not limited thereto, I shall now give a typical example of procedure leading to a grease-proof paper product which resists for very long periods of time penetration by grease, for instance, when put to such exacting service as the liner bag of a two-ply paper bag for holding and vending ground coffee. Such procedure will be described with reference at the appropriate time to the accompanying drawing, whereof Figure 1 illustrates diagrammatically and conventionally preferred instrumentalities, including a pair of rolls, for applying the zein solution to the primed paper sheet and Figure 2 represents a fragmentary section through the rolls as the paper sheet is passing therebetween and is receiving a coating of the zein solution.

The paper base used as the starting material may be a rosin-sized kraft paper sheet of the ordinary wrapping paper type composed of well-beaten pulp and having a basis weight of, say, about 20 to 30 pounds (i. e., the weight in pounds of a ream of 480 sheets, 24" x 36"). The expression "well-beaten pulp" as used herein means that, although the pulp has been beaten to a stage well beyond that customary in the manufacture of, say, ordinary wrapping paper, it is none the less at a stage of hydration or gelatinization far short of that developed in glassine paper manufacture. The sheet may be run continuously either from a roll accumulation or from the dry end of a papermaking machine through an ordinary size-press or tub containing the priming composition hereof. A satisfactory priming composition for the purposes hereof may consist of an aqueous suspension of about 3% bentonite and about 3% cooked potato starch. The size-press may be operated to apply the priming composition to either or both faces of the sheet. Ordinarily, however, it is desirable to apply the priming composition to both faces of the sheet, since the composition is comparatively inexpensive and only a very small amount need be deposited on the sheet and infused into its surface pores. In such latter case, the sheet may be progressively led through the bath of priming composition and thence into the nip of the press rolls forming part of the size-press. Pursuant to such operation, the sheet as it issues primed on both its faces from the size-press may have taken up about 0.5% to 2% bentonite and about 0.5% to 2% starch, based on the dry weight of the starting sheet.

The primed sheet issuing from the size-press may be dried on the usual steam-heated drier drums, whereupon it may be calendered in the customary way to acquire a smooth or polished surface. The dried, primed paper sheet may then be wound into rolls for transfer to the zein-coating machine, although in some cases such sheet may be led directly from the drier drums or calender to the zein-coating machine. A highly satisfactory zein-coating machine is one comprising a pair of squeeze rolls into whose nip the primed sheet is progressively passed. The zein solution is added to the upper face of the sheet at the nip, a small bank of solution being constantly maintained at the front or ingress of the nip. It is desirable to prevent a coating of dried zein from building up on the upper roll periphery by reason of evaporation of solvent from the film of zein solution remaining on such periphery as the sheet leaves it. While this may be done by housing the upper

roll in a suitable metal enclosure, it is accomplished simply and advantageously, as illustrated in Figure 1, by causing the paper sheet as it leaves the nip to wrap over the top roll for as much of its periphery as possible, preferably a peripheral surface of about 180° or more.

It will be observed from Figure 1 that the primed paper sheet S is progressively passed at an angle upwardly into the nip of the press rolls 10 in front of which is maintained a small bank B of the zein solution. The zein solution may be continuously fed onto the upper paper surface from a nozzle 11 whose discharge end 12 is disposed substantially centrally and immediately in front of the nip and slightly above the paper surface. The solution may be carefully metered or regulated in its flow onto the paper so as to maintain the bank B of substantially constant size sufficient to coat the paper sheet substantially uniformly throughout its entire width or upper surface and at the same time to avoid appreciable overflow or extrusion of solution beyond the paper edges. It is preferable that one of the two rolls 10 be peripherally covered with a yielding or resiliently soft substance, for example, soft rubber, and that the other roll present a hard peripheral surface, for example, a smoothly polished steel surface. As shown, the lower roll has a soft-rubber periphery 10a, whereas the upper roll has a smooth steel periphery. The upper roll may be urged or pressed against the paper by a dead weight or by springs in the usual manner.

The soft-roll periphery ensures uniform pressure between the paper sheet and the hard roll-periphery and thereby fosters the deposition of a substantially uniform coating of zein solution on the preferably primed paper sheet. When it is realized that a paper sheet normally varies in thickness at least a fraction of a thousandth of an inch and that the zein coating is of a thickness amounting to a fraction of a thousandth of an inch, the desirability of providing substantially uniform pressure over the entire upper sheet surface, as it is being coated with zein solution, is at once recognized.

It is highly desirable that the sheet entering the nip between rolls 10, 10 wrap the lower roll for a material distance so as to seal the edges of the paper sheet and thereby prevent the coated solution from running under the sheet edges. If such running of coating solution under the sheet edges were permitted, not only would needless waste of relatively expensive coating solution be occasioned, but the roll of paper sheet finally accumulated at the end of the zein-coating machine would lack uniformity in that the edge portions of the sheet would be much harder than the rest of the sheet; and the edge portions would tend to stick together or "block" with attendant difficulty in unwinding the sheet from the roll.

As illustrated in Figure 1, the sheet S, as it is being coated with the zein solution, wraps the lower roll 10 so that the bank of coating solution 13 cannot creep under the sheet edges; and such wrap of the lower roll by the sheet is over a substantial arc, say, upwards of about 10°, the particular arcuate angularity or extent of the wrap depending upon the size of the roll. In order to realize maximum benefit from the wrap on the lower roll 10, it is desirable to station the two rolls with their axes in the same vertical plane or with the axis of the upper roll somewhat offset in the direction of travel of the paper sheet 75 through the nip. The long wrap of the paper

sheet about the upper roll periphery avoids such long-time exposure of the residual film of zein solution on such periphery as would be attended by drying and setting of such film.

Although zein solution as it is applied to the paper sheet may vary in its concentration and contain various volatile organic solvents of zein, it preferably consists of a zein solution of about 20% to 25% strength or concentration in ethyl alcohol. Such a solution has a consistency or viscosity appropriate for coating at about room temperature the preferably primed paper sheet by the particular and advantageous method just described. The conditions of coating are preferably such as to deposit the zein on one face of the paper sheet in amount of only about 1 to 2 pounds per ream (2880 square feet) of paper. Indeed, with an appropriate base paper sheet and an appropriate priming treatment, it is possible to arrive at the greaseproof quality desired in the finished paper product hereof with a zein coating composition applied to only one face and amounting, on a dry basis, to as low as about 0.4 pound of such composition per ream of paper. The paper sheet thus thinly coated with zein solution may be progressively run through an air-drier, for instance, through a warm-air tunnel, to promote complete removal of the ethyl alcohol solvent. The resulting zein-coated paper sheet may then be wound in rolls and shipped to the consumer. It has been found that when such sheet is used as the liner bag of a two-ply paper bag for holding ground coffee, its greaseproofness is such that no stain is visible on the exterior surface of the liner even after its interior or zein-coated surface has been in contact with its ground coffee contents for many months. It might be noted that the greaseproof paper product hereof can be handled in the usual bag-feeding, bag-folding, and pasting equipment without the slightest difficulty; and the finished bag may without danger of tearing or other difficulty be filled with coffee or other comestibles by automatic bag-filling machinery. It will be appreciated, of course, that the paper product herein might be coated with zein on both its faces, but it is usually desirable from the standpoint of economy to coat with zein only the face of the paper product to come into contact with greasy or oily comestibles.

In one example of procedure, kraft pulp was beaten to a Canadian freeness of 350 cc. and then was converted into 25-pound paper (weight per 2880 sq. ft.) in the conventional way on a Fourdrinier machine. The paper showed an oil resistance of only 5 seconds on the wire side and 15 seconds on the top or so-called web side. The sheet was then passed through a size press wherein it was treated with an aqueous mixture of bentonite and cooked potato starch containing 3% of each. After it had been redried it showed an oil resistance of 35 and 110 seconds on the "wire" and "web" sides, respectively. The oil-resistance values were determined by noting the time for lubricating oil of S. A. E. viscosity 30 to break through the sheet over about 90% of the surface of 1 inch square specimens floated on the oil at 70° F. A zein solution was then applied to the web side of the bentonite treated sheet, and, although only 1.7 pounds of dry coating was deposited per ream (2880 sq. ft.), the sheet was substantially oil-and-turpentine-proof. The "web" side of the sheet was coated, since this side usually gives the better result with regularity. In a second case, the pulp was beaten to

5 a freeness of 225, the 28-pound paper made from it had an oil resistance of 25 seconds on the wire side and 90 seconds on the web side, prior to the bentonite-starch tubbing, and an oil resistance of 70 and 250 seconds on the corresponding sides after the tubbing and redrying. When the web side was coated with only 1.2 pounds, dry basis, of a mixture of 3 parts of zein and 1 part of invert sugar deposited from an alcohol solution 10 containing a small proportion of water, it was substantially oil-and-turpentine-proof. When to the bentonite-starch tubbing mixtures a little ammonia water or equivalent deflocculating agent is added, the oil resistance of the tubbed sheet is even higher than above indicated. In 15 any case, it is significant that the ash-content of the paper was increased less than about 1 1/4% when the sheet was primed with the bentonite-starch mixture, and that no coating of bentonite 20 or starch was visible on the paper prior to its being coated with zein.

In lieu of bentonite, it is possible to use for the purpose of priming the paper surface an appropriately colloidal clay, preferably a colloidal clay 25 that has been additionally peptized in water containing ammonia or equivalent clay deflocculating agent. The use for the paper-priming purposes hereof of the colloidal fraction of china clay, for instance, such fraction as is separated 30 from the whole clay by an electrophoretic fractionating method, together with ammoniated water as the suspending medium for such fraction leads to results somewhat similar to those had from bentonite; and the term "bentonite" as used 35 in the appended claims is meant to include such colloidal clay fraction. However, bentonite as such is generally to be preferred because of its lower cost and the consistently excellent results realized therefrom. Again, it is possible to use 40 in lieu of zein on the bentonite-primed paper surface such other grease-resistant, film-forming, solid substances as nitrocellulose, acetylcellulose, other cellulose esters, various cellulose ethers, etc. Such grease-resistant, film-forming substances 45 may, as in the case of the zein, be applied to the primed paper sheet as solutions in suitable volatile organic solvents. However, grease-resistant prolamines, such as zein, are highly effective and economical when used 50 accordanit with the present invention; and the greaseproof coating or film afforded thereby on the preferably primed paper surface is characterized by the firmness or high tenacity of its bond with the primed paper surface, insomuch 55 that such coating or film has practically no tendency to peal or break away from the paper base in the course of handling the greaseproof paper product hereof or of fabricating it into liner bags, liners, etc.

60 Because of the extreme thinness of the zein coating solution on the preferably primed paper sheet hereof, the tendency for curling of such paper sheet during its drying is minimized. Such minimization of curling is especially important 65 in the case of thin or lightweight paper bases, whose resistance to curling is low, especially when the finished paper product hereof is intended to be cut into flat sheets or blanks for lining paper-board boxes. It is, moreover, possible to incorporate into the zein solution plasticizing agents, such as invert sugar, glycerine, ethylene glycol, and other substantially non-volatile alcohols or glycols that serve to offset curling tendency in 70 the finished paper product hereof.

The zein-coated paper product hereof lends

itself particularly well to coating very thinly with wax, such as paraffin, to yield a paper product highly resistant to the passage of water vapor therethrough. Thus, the paper product hereof may be made remarkably moistureproof as well as 5 greaseproof by being coated on its zein-coated face with molten paraffin wax or its equivalent in amount as little as about 2 to 4 pounds of paraffin wax per ream. The reason why such small amounts of wax are effective in contributing 10 high moisture-impermeability to the waxed paper product hereof is because the zein coating on such product keeps the paraffin wax practically entirely on the paper surface, that is, prevents the wax from being dissipated into the 15 body of the paper sheet. In some instances, it may be desirable to produce a paper product waxed on both its faces, as by running the zein-coated base paper sheet through a bath of molten paraffin wax. In such instances, the preferably 20 primed paper sheet is advantageously coated with the zein composition on both its faces, as by running the preferably primed paper sheet through a bath of the zein coating composition or by spreading such composition first on one face and then on the other. The resulting paper product waxed on both its faces may carry no more than about 25 2 to 4 pounds of paraffin wax per ream of paper in acquiring the desired high moistureproofness. It might be noted that the application of the zein composition and wax to both surfaces of the paper sheet minimizes tendency for the paper product to curl, since such shrinking or curling forces as may be incident to the application of the zein composition and/or wax to one face of the sheet are substantially neutralized by similar forces incident to the application of the zein composition and/or wax to the other face of the sheet.

The improvement in the oil or grease-resistance of the base paper effected by the bentonite-starch composition or "tubbing" is important because it makes possible, by keeping the film-forming medium practically entirely on the surface, the attainment of substantially complete 30 imperviousness with an exceedingly small quantity of film-forming material.

Extensive research and investigation of the factors underlying the results secured pursuant to the present invention have led to the conclusion that contributing importantly to these results are three factors or aspects, namely, the hydration of the pulp entering into the base sheet, the priming composition, and the zein or equivalent prolamine coating composition. Thus, well-beaten or well-hydrated cellulose pulp or 35 papermaking stock makes possible the realization of a paper sheet or base whose texture or density is appropriate for yielding, upon being primed with the bentonite-binder composition, a finished paper sheet of the desired greaseproof quality even when the greaseproofing zein coating composition is extremely thin or attenuated, for instance, is spread on one face of the paper sheet in amount ranging from only about 0.4 to 40 2 pounds of the dry zein composition per ream (2880 square feet) of paper. Because the dried zein composition exists in such attenuated or thin film form on the primed paper base, whose content of priming solids is also very low, it becomes possible to produce greaseproof paper products 45 strongly competitive even with glassine paper, for such greaseproof paper products exhibit flex-enduring and tear-resisting qualities markedly superior to those of glassine paper.

The valuable factor of priming the base sheet need not, however, necessarily be utilized, provided that the factor of beating or hydrating the pulp entering into the paper sheet or base is appropriately correlated with the aspect of the zein-coating composition to foster the greaseproof quality desired in the finished paper product along with such other qualities as the desired high flex-endurance and tear-resistance. Thus, the priming treatment may be omitted, even in the case of relatively thin or lightweight papers, for instance, those having a basis weight ranging from, say, about 15 to 35 pounds, when the kraft or other cellulose pulp entering into the paper sheet or base has been appropriately beaten, that is, to a stage of hydration distinctly greater than that of the pulp used in ordinary kraft wrapping paper manufacture but far short of that of the pulp used in glassine paper manufacture. In such latter instance, one need not, in realizing the highly greaseproof paper products hereof, spread more zein coating composition than that already indicated as yielding a very thin or highly attenuated film on the paper base, for instance, zein coating composition amounting on a dry basis to no more than about 0.4 to about 2 pounds per ream surface (2880 square feet). As already indicated, such a very thinly zein-coated paper product has the desired high flex-enduring and tear-resisting qualities coupled with the desired greaseproofness.

The terms "greaseproof" or "grease-resistant," as used in the foregoing description and in the appended claims in characterizing a paper product hereof, mean that such product shows no sign of oil-staining or oil-leakage when such product is subjected to the so-called turpentine test. This test is conducted by supporting the paper product specimen with its zein-coated face up on a sheet of white absorbent paper, placing on such upper face a small mound of fine sand, and adding to the sand a slight excess of moisture-free turpentine containing a small amount of a suitable dye. After about 4 to 6 hours, the specimen is lifted from the underlying absorbent paper support. Should the absorbent paper support display no sign of staining by the dyed turpentine, the specimen is considered to be greaseproof. It might be noted, however, that the 45 greaseproof or grease-resistant paper products hereof usually are vastly more grease-resistant or greaseproof than that necessary to satisfy such conventional test. Indeed, the products hereof usually show no transmission therethrough of turpentine even after a test period of about 12 to 16 hours.

I claim:

1. A grease-resistant paper product primed on its surface with bentonite and cooked starch and 50 filmed on such primed surface with grease-resistant prolamine.
2. A grease-resistant paper product comprising a substantially non-grease-resistant paper base primed on its faces with a mixture of bentonite and binder and filmed on at least one primed face with grease-resistant prolamine.
3. A grease-resistant paper product primed on its surface with bentonite and cooked starch and 55 filmed on such primed surface with zein in amount of only about 0.4 to 2 pounds per ream surface (2880 square feet).
4. A grease-resistant paper product comprising a substantially non-grease-resistant paper base primed on its faces with a mixture of bentonite and cooked starch and filmed on at least 60

one primed face with a film containing grease-resistant prolamine as an essential constituent, said film being present in amount of only about 0.4 to 2 pounds per ream surface (2880 sq. ft.).

5. A grease-resistant paper product primed on its surface with bentonite-binder composition and filmed on such primed surface with zein, said zein containing a plasticizing agent.

6. A grease-resistant paper sheet primed on its surface with bentonite-binder composition and filmed on such primed surface with zein, said zein containing invert sugar.

7. A paper sheet of high grease-resistance and low water-vapor penetrability, said sheet being primed on its surface with bentonite-binder composition, being filmed on such primed surface with zein, and being waxed over said zein.

8. A paper sheet of high grease-resistance and low water-vapor penetrability, said sheet being primed on its surface with bentonite and cooked starch, being filmed on such primed surface with zein in amount of only about 0.4 to 2 pounds per ream surface (2880 square feet), and being waxed over said zein with only about 2 to 4 pounds of wax per ream surface.

9. A process of producing a grease-resistant paper product, which comprises priming the surface of a paper base with an aqueous composition containing bentonite and water-soluble binder, drying the primed surface, filming the primed surface with an alcohol solution of zein, and drying the filmed surface.

10. A process of producing a grease-resistant paper product, which comprises priming the surface of a paper base with an aqueous composition containing bentonite and cooked starch, drying the primed surface, filming the primed sur-

face with an alcohol solution containing zein as an essential constituent in amount to deposit only about 0.4 to 2 pounds of filming substance per ream surface (2880 square feet), and drying the filmed surface.

11. A process of producing a grease-resistant paper product, which comprises priming the surface of a paper base with an aqueous composition containing bentonite and cooked starch, drying the primed surface, filming the primed surface with an alcohol-water solution of zein and invert sugar, and drying the filmed surface.

12. A process of producing a paper product of high grease-resistance and low water-vapor penetrability, which comprises priming the surface of a paper base with an aqueous composition containing bentonite and water-soluble binder, drying the primed surface, filming the primed surface with a volatile organic solvent solution of zein, drying the filmed surface and waxing the dried, filmed surface.

13. A greaseproof paper product which is especially adapted for wrapping and packaging greasy and oily comestibles and whose paper base is composed essentially of cellulose pulp in thoroughly beaten state greater than that of the pulp used in kraft wrapping paper manufacture but far short of the gelatinized state of pulp entering into glassine paper manufacture, said base being of a weight ranging from about 15 to 35 pounds per ream surface (2880 square feet) and being filmed with prolamine in amount of only about 0.4 to 2.0 pounds per ream surface, said product exhibiting flex-enduring and tear-resistant qualities markedly superior to those of glassine paper of similar basis weight.

MILTON O. SCHUR.